

## UNITED STATES PATENT OFFICE

2,113,423

LIGHT SENSITIVE PAPER AND METHOD OF  
TREATING SAME

Clyde A. Crowley, Chicago, and George H. Goodyear, Evanston, Ill., assignors to The Huey Company, Chicago, Ill., a corporation of Illinois

No Drawing. Application April 30, 1937,  
Serial No. 139,950

## 4 Claims. (Cl. 95—6)

Our invention relates to light-sensitive paper and to a predeveloper therefor, and particularly relates to a novel coating for blue print paper and to a chemical compound adapted for use in the treatment thereof.

A developer of the type intended for use in the described relation is disclosed in our Patent No. 2,093,421, September 21, 1937.

One of the principal problems in the manufacture of blue print paper is that of providing a coating therefor having a known stability or permanency under adverse climatic conditions; in other words a paper that the manufacturer may distribute with the assurance that it will remain effective for at least a known period, preferably over one year. The desire, and in many cases the necessity for a certain degree of permanency has been responsible for the general use of a coating compound that is relatively slow in action and which does not produce bright or intense blue color without bleeding and the resultant partial obliteration of the white lines. An object of our invention is, therefore, to provide a perfectly stable coating, one that operates to completely eliminate bleeding in development and one in which an intense blue is present in the final product, and a paper which prints at greater speed than products heretofore known.

The improvement is brought about by the use of a novel coating containing some of the usual components, but in which a substance that acts as a catalyst to accomplish the needed results, is incorporated. The catalytic agent which we have discovered is ammonium nitrate.

Although the above catalyst may be added to the known types of blue print sensitizing solutions with beneficial results, in practice we prefer to formulate sensitizing solutions particularly adapted to take advantage of the catalytic reaction induced by this substance.

One sensitizing solution that has been found to be appropriate and satisfactory is as follows, the formula providing for a bath of approximately five (5) gallons.

1. Potassium carbonate oz. 11  
2. Oxalic acid oz. 11  
3. Ammonium nitrate oz. 8  
4. Ferric ammonium oxalate lbs. 8  
5. Potassium ferricyanide oz. 6  
6. Water, to bring the solution to 14.5° Bé.

A paper sensitized with the above solution will not produce good prints when developed in the ordinary manner, due to its low potassium ferricyanide content. If a special predeveloper of the

type described in our U. S. Patent No. 2,093,421 and hereinafter described, is not used, the color is not sufficiently deep.

However, when a paper coated with the above type of sensitizer is treated with this special type of predeveloper, an exceptionally fine print will result. For example, the so-coated sheet should be developed in a solution such as the following and then be washed and treated with an oxidizing solution and rinsed.

|                           |                                                               |
|---------------------------|---------------------------------------------------------------|
| 1. Potassium carbonate    | oz. 10                                                        |
| 2. Oxalic acid            | oz. 8.5                                                       |
| 3. Disodium phosphate     | (Na <sub>2</sub> HPO <sub>4</sub> .12H <sub>2</sub> O) oz. 22 |
| 4. Glucose                | oz. 5.5                                                       |
| 5. Potassium ferrocyanide | lbs. 7                                                        |
| 6. Sodium bisulphite      | oz. 13.5                                                      |
| 7. Water, to make         | gals. 5                                                       |

A number of other satisfactory predeveloper solutions are disclosed in our said Patent No. 2,093,421. Another satisfactory solution is as follows:

|                           |                                                               |
|---------------------------|---------------------------------------------------------------|
| 1. Potassium carbonate    | oz. 11                                                        |
| 2. Oxalic acid            | oz. 9.5                                                       |
| 3. Disodium phosphate     | (Na <sub>2</sub> HPO <sub>4</sub> .12H <sub>2</sub> O) oz. 24 |
| 4. Sucrose                | oz. 8                                                         |
| 5. Potassium ferrocyanide | lbs. 8                                                        |
| 6. Sodium bisulphite      | oz. 12                                                        |
| 7. Water, to make         | gals. 5                                                       |

When the exposed paper is washed in a solution such as above defined, the excess of ferrous iron in the exposed portions reacts with the ferrocyanide of the predeveloping solution to form ferro-ferrocyanide. The concentration of the ferrocyanide ion in the developer is great enough so that no ferrous iron has the opportunity to wash or bleed due to the insolubility of ferrous ferrocyanide.

The exposed paper is then given the customary water wash, bichromate wash and water rinse.

When in use, this predeveloper gives better results if the oxidation of the ferrocyanide is inhibited by the presence of a reducing agent, but this reducing agent must not be strong enough to reduce the iron in the ferric complex on the paper. In practice, sodium bisulphite has been found satisfactory.

A further improvement in the brilliance of the print is achieved by decreasing the particle size of the pigment on the paper. This is done by means of aliphatic polyhydroxyl compounds, aliphatic aldehydes and aliphatic ketones incorpo-

rated in the predeveloper which will not react with iron salts to form insoluble reaction products. In practice, various sugars are satisfactory.

5 In order to obtain good whites with the ferrocyanide predeveloper, it is necessary to buffer the acid concentration rather carefully. Any of the common acid buffers are satisfactory, provided they do not have too powerful oxidizing 10 or reducing properties. In use are mixtures of potassium oxalate, potassium acid oxalate and oxalic acid or mixtures of sodium acid phosphate and oxalic acid.

15 It will be noted that the catalyst constitutes a small but definite component in the sensitizer disclosed.

Although the specific chemical or chemical-physical mechanism is not understood, it is believed that the action is catalytic for reasons 20 which are enumerated. This catalyst may be incorporated with the known type of sensitizing solution as follows:

|                            |       |    |     |
|----------------------------|-------|----|-----|
| 1. Ammonium nitrate        | ----- | g  | 3   |
| 2. Citric acid             | ----- | g  | 6   |
| 3. Ammonium oxalate        | ----- | g  | 6   |
| 4. Ferric ammonium oxalate | ----- | g  | 42  |
| 5. Potassium ferricyanide  | ----- | g  | 7.5 |
| 6. Water, to make          | ----- | cc | 250 |

30 This formula is for development in the customary manner involving washing and treatment with an oxidizing agent.

In all cases the inclusion of the catalyst improves the speed and the blue color, improves 35 the ease of washing the paper and stabilizes the sensitizing solution against deterioration during storage, as well as stabilizing the paper thus

coated against rapid spoiling under normal or adverse atmospheric conditions.

The possible actions of the catalyst above disclosed in effecting the results described have been 5 the subject of extensive laboratory study aimed at determining the probable mechanism by which these substances produce the desirable effects described. Observations as made, in our opinion, restrict the action of the substance claimed to the field of catalysis.

We claim:

1. The method of making blue prints which 15 consists in coating a paper with a solution comprising a light-reduceable ferric complex, a ferricyanide salt and ammonium nitrate as a catalyst that will stabilize said coating, then exposing parts of said paper to light and then treating said paper in a predeveloper comprising an acid reacting water solution of a ferrocyanide.

2. The method of making blue prints which 20 consists in coating a paper with a solution comprising a light reduceable ferric complex, a ferricyanide salt and ammonium nitrate, then exposing parts of said paper to light and then developing said paper.

25 3. The method of making blue prints which consists in coating a paper with a solution comprising a light-reduceable ferric complex, a ferricyanide salt and ammonium nitrate, then exposing parts of said paper to light and then treating said paper in a predeveloper comprising an acid reacting water solution of a ferrocyanide.

4. A coating for blue print paper comprising a light-reduceable ferric complex, a ferricyanide salt and ammonium nitrate.

CLYDE A. CROWLEY.

GEORGE H. GOODYEAR.